

## UNITED STATES PATENT OFFICE

2,308,185

## ADHESIVE COMPOSITION

Wesley N. Lindsay, Brooklyn, N. Y., and Harold Charles Lietz, San Francisco, Calif., assignors to The Arabol Manufacturing Company, New York, N. Y., a corporation of New York

No Drawing. Application August 23, 1940,  
Serial No. 353,892

3 Claims. (Cl. 106—157)

This invention relates to adhesive compositions, and more particularly to improved adhesives of the class containing gel forming protein, commercially termed "iceproof glue."

The adhesive of the present invention is useful for attaching paper labels and the like to containers, characteristic in that immersion in cold water does not disturb the adhesion of the label. Generally speaking, the iceproof glue or adhesive is used to attach relatively water permeable members, such as paper labels or the like, to reusable containers such as bottles. The labeled container may be immersed in cold or iced liquid over fairly long periods, the label firmly remaining on the bottle, not being removable by ordinary handling. A further general characteristic of iceproof glue is that a label attached therewith may be readily removed from the container by washing with warm water, even without the use of a detergent.

Iceproof glues are well known in the art and are in rather extensive use. They contain an animal glue or similar gel forming protein in water soluble form, in a concentration which would set to a firm gel in the absence of modifying substances. They also contain a highly water soluble substance which may be termed a "gel inhibitor" or "liquefying agent." The inhibitor or agent is one which does not react with protein or alter its chemical structure to render it incapable of gelation. Its function is to inhibit the gelation or lower the temperature at which gelation occurs. When the agent is removed from the protein solution it leaves it in such condition that gel formation thereupon occurs.

The action or operational mechanism of iceproof glue is as follows: The adhesive film between the label and container contains the soluble protein and liquefying agent in combination, as previously stated. The label becomes permeated with water upon immersion in cold water. The highly water soluble liquefying agent rapidly dissolves, and diffuses through the label. The concentration of liquefying agent in the adhesive film thereupon becomes reduced, and gelation of the protein is no longer inhibited. A gel is formed which can only extremely slowly disperse or dissolve in water. The gel has sufficient adhesive properties to adhere the label effectively onto the container. The gel so formed may however be liquefied by heat. Thus, washing the label at

an elevated temperature readily effects a complete and clean removal of the label from the container.

Iceproof glue generally contains other ingredients than those mentioned. Starch, dextrine, or other modified starch is generally included to increase the initial viscosity or tackiness of the glue, and otherwise improve its operation with labeling machinery, or the like. It also decreases stringiness in the glue. The starch may be added to the adhesive composition in its modified form. On the other hand, it may be added directly and modified in the process of manufacturing the adhesive. Another ingredient is generally added to decrease the rate at which the dry glue film is permeated and swollen by cold water. A readily dispersable non-aqueous and water insoluble substance of relative high viscosity, such as lanolin, effects the latter characteristic therein. Still other ingredients may be included in the glue, such as to preserve it from bacterial attack, and for other purposes well known to those skilled in the art.

Among gel inhibitors or liquefying agents previously used or proposed for iceproof glues are calcium chloride, calcium nitrate, magnesium chloride, sodium chloride, sodium nitrate, urea and lactic acid. However, the prior liquefying agents rendered the iceproof glue either so hygroscopic as to present greatly retarded drying rates under high humidity; or, decreased its "iceproofness" by permitting the liquefied protein to dissolve too rapidly and diffuse through the label.

In accordance with the present invention, the use of a water soluble thiocyanate is proposed as the liquefying agent for animal glue gels, and particularly for application in adhesive of the iceproof glue type. We have found that the use of water soluble thiocyanate overcomes the disadvantages of the prior liquefying agents. The adhesive composition of the invention is neither too hygroscopic nor too stable in its liquefaction. The adhesive composition or iceproof glue of the invention contains a water soluble thiocyanate as the liquefying agent, the other ingredients being similar to those of the prior art compositions. We have found that the composition of the invention may be readily adapted for all commercial applications for such adhesives, re-

maining stable under widely varying conditions. By way of example, the following typical compositions are given:

*Example I*

|                       | Pounds  |
|-----------------------|---------|
| Animal glue (360 gm.) | 120     |
| Ammonium thiocyanate  | 50      |
| Tapioca starch        | 120     |
| Water                 | 259     |
| Phenol                | 1       |
| <br>Total             | <br>550 |

*Example II*

|                       | Pounds  |
|-----------------------|---------|
| Animal glue (360 gm.) | 105     |
| Sodium thiocyanate    | 52      |
| Sago starch           | 105     |
| Water                 | 267     |
| Lanolin               | 20      |
| Phenol                | 1       |
| <br>Total             | <br>550 |

The proportions of the ingredients may of course be considerably varied. The procedure of preparing the adhesive composition is similar to that heretofore practiced, and well known by those skilled in the art. Briefly, the animal glue is mixed with the water and allowed to stand for one hour without heating. The mixture is then raised to a temperature of about 55 to 60° C. to complete the dispersion of the glue and the liquifying agent, namely the thiocyanate, is added to the mixture at about this temperature. The starch which may have been previously moistened with a portion of the water component, is then added to the mixture at the elevated temperature. The mixture is then agitated and heated in a temperature of 65 to 70° C. and the remaining ingredients of the composition are added. The resultant adhesive is then strained, if necessary, and cooled. In an alternate procedure, the starch is added in a dry state providing the liquified glue mixture is cooled from its 55 to 60° C. temperature to about 45° C. to inhibit "lumping."

Suitable commercial water soluble thiocyanates are those of ammonium, sodium and potassium, although others may be used. Practical proportions of the thiocyanate is in the range of 25 to 60 per cent of the dry weight of the glue. Other starches than the tapioca and sago starches illustrated, may be used; as may dextrines or modified

starches. The characterization of the animal glue ingredient by its "gram strength," e. g. (360 gm.), is common in the art and reference to the standard test used to evaluate the gel strength or hardness of glue. The invention, of course, is not limited to any particular protein glue or "gram strength" thereof. A wide variety of animal glue, gel forming proteins, and gelatin may be used by suitably varying the formula of the composition to produce the desired results. The purified gelatin may be substituted. The protein used must have gel forming characteristics in aqueous solution which is inhibited or depressed by the liquifying agent.

15 Although specific compounds and compositions for practicing the invention have been described and illustrated, it is to be understood that modifications which fall within the broader spirit and scope of the invention may be practiced, and accordingly we do not intend to be limited except as set forth in the following claims.

What we claim is:

1. An iceproof glue of the character described comprising the combination of a gel forming protein and starch in substantially equal proportions, and a water soluble thiocyanate in the proportion of about 60 per cent of the dry weight of said protein to inhibit gel formation of the protein in the composition, said thiocyanate dissolving out of 20 the composition when it is immersed in water to effect gel formation of said protein therein.

2. An iceproof glue of the character described comprising the combination of a protein which disperses in hot water and gels upon cooling, 25 starch substantially equal in amount to said protein, and a water soluble thiocyanate in the proportion substantially in the range of about 25 to 60 percent of the dry weight of said protein for inhibiting the gel formation of the protein and 30 gelatinizing and stabilizing dispersion of the starch in the glue.

3. An iceproof glue of the character described comprising the combination of a gel forming protein, starch substantially equal in amount to said 35 protein, lanolin, water, and an alkali thiocyanate substantially in the range of about 25 to 60 percent of the dry weight of said protein for inhibiting the gel formation of the protein and 40 gelatinizing and stabilizing dispersion of the starch in the glue.

WESLEY N. LINDSAY.  
HAROLD CHARLES LIETZ.